

## UNITED STATES PATENT OFFICE

2,097,211

## PROTECTIVE TREATMENT OF METALS AND ALLOYS

Herbert Tasman Davies, London, England, assignor to The Metallurgical Treatment Syndicate Limited, Edinburgh, Scotland

No Drawing. Application July 18, 1935, Serial No. 32,117. In Great Britain August 13, 1934

4 Claims. (Cl. 148—6.5)

This invention relates to a protective treatment for metals and alloys particularly iron and steel for the purpose of rendering them incorrodible. More particularly the present invention relates to that class of treatment in which phosphoric acid or a phosphate salt solution is used to produce a coating or integral surface layer of phosphate.

To facilitate the formation of phosphate coatings it has been proposed to deposit iron or zinc electrolytically prior to the phosphate treatment.

According to the present invention I treat articles to be rendered incorrodible prior to the phosphate treatment for a short period of say a few seconds to a few minutes with a dilute solution of a salt of copper and/or of nickel; simultaneously or prior to such treatment I may treat the articles with a solution of a zinc salt.

The treatment or treatments may be an immersion at ordinary room temperature or at a somewhat raised temperature, but preferably an electric current is employed to facilitate or hasten the action, the article to be treated being made a cathode.

The effect of the treatment or treatments seems to be to prepare an advantageously smooth surface on the foundation metal so that the subsequent treatment in a bath of iron phosphate or phosphoric acid with or without added iron or iron phosphate in the known manner ensures an improved union of the resultant phosphate coating with the foundation metal and an improved incorrodibility.

In the case, for example, of carrying out the invention upon an iron or steel article it may be immersed in a bath of copper and/or nickel sulphate solution of about one per cent. strength and made the cathode for an electric current for a period of from a few seconds to a few minutes, the time being to some extent dependent on the strength of the solution and the temperature. If a composite treatment is desired, a similar treatment in a zinc sulphate bath may precede the treatment in the copper and/or nickel sulphate bath, or the zinc sulphate may be added to the copper and/or nickel sulphate bath.

The article thus pretreated is then given the phosphate coating by treatment in a bath containing merely phosphoric acid or iron phosphate or both with or without metallic iron or I may employ a bath of mixed phosphates, the added metallic phosphate, for example chromium nickel or copper phosphate, serving to cause the formation of a deposit or coating of

mixed phosphates having good protective properties in relation to the iron or steel.

In the case of treating the article with a zinc salt solution as well as with the copper or nickel salt solution I may use a simple zinc salt solution or I may use a solution of zinc sulphate containing small amounts of common salt, boric acid, aluminium sulphate, and dextrine.

Subsequent to the production of the phosphate deposit the corrosion resisting qualities of the treated metal may be further improved by the adoption of the well-known process of oil immersion either at ordinary or elevated temperatures, the excess of oil being removed.

What I claim is:—

1. A protective treatment for metallic articles consisting essentially of iron comprising subjecting said articles to the action of a solution of about one per cent strength of a water-soluble salt of a metal taken from the group consisting of copper and nickel for a period ranging from a few seconds to a few minutes while simultaneously passing an electric current through the solution using the article as a cathode, and then treating the article to formation of a metallic phosphate coating.

2. A protective treatment for metallic articles consisting essentially of iron comprising subjecting said articles as the cathode of an electric circuit to the action of a solution of a water soluble copper salt of about one per cent. strength for a period ranging from a few seconds to a few minutes and then forming thereon a metallic phosphate coating.

3. A protective treatment for metallic articles consisting essentially of iron comprising subjecting said articles as the cathode of an electric circuit to the action of a solution of about one per cent strength of a mixture of water soluble nickel and copper salts for a period ranging from a few seconds to a few minutes and then forming thereon a metallic phosphate coating.

4. A protective treatment for metallic articles consisting essentially of iron comprising subjecting said articles as the cathode of an electric circuit to the action of an aqueous solution of a zinc salt, simultaneously to the action of an aqueous solution of a salt of a metal taken from the group consisting of copper and nickel, the metallic salt solution being of about one per cent strength and finally subjecting the articles to the formation of a metallic phosphate coating.

HERBERT TASMAN DAVIES.